

## UNITED STATES PATENT OFFICE

2,093,377

## PRINTING WITH MORDANT DYESTUFFS

Heinrich Werdenberg, Neu-Allschwil, near Basel,  
Switzerland, assignor to the firm Durand &  
Huguenin S. A., Basel, Switzerland

No Drawing. Application March 16, 1934, Serial  
No. 716,001. In Germany March 20, 1933

## 3 Claims. (Cl. 8—6)

It is known that in printing natural or artificial silks with chrome dyestuffs the printed parts of the material acquire an undesired harsh feel and the lustre of the fibre is much diminished. 5 These effects appear to be due in some cases to the fact that certain thickening agents undergo coagulation; with the chrome mordant (chrome acetate) this is particularly so in the case of gum thickening, which otherwise is especially 10 well suited for printing on silk. The aforesaid disadvantage is present not only in printing on silk or artificial silk, but under some circumstances and in a smaller degree also in printing on other fibres such as wool, wool-like material 15 and cotton. For the latter fibre for instance arabic gum thickening would be well suited for handprinting as this thickening matter gives very sharp prints even in the finest designs. But up to the present time it has not been possible 20 to use arabic gum thickening and the usual chromium mordant—chromium acetate—in a printing paste, because this latter is not stable (coagulation takes place) and the prints obtained present a harsh feel. 25

In U. S. Patent No. 1,942,774 there is described a process for printing with chrome dyestuffs on natural silk, wherein the printing paste contains besides the usual ingredients (dyestuff, chromium acetate) urea, a soluble sulphocyanide 30 and an aliphatic poly-alcohol. In this process the soft feel and normal lustre of the printed fibres are retained even when gum thickening is used in the printing paste.

Whilst this process does indeed yield good results in printing on natural silk, it is less suited for printing on other fibres, such as artificial silk (viscose). On viscose it is possible to produce prints which are satisfactory with respect to the feel and lustre of the printed parts only under 40 certain circumstances, by special selection of the thickening agent and by using urea without a sulphocyanide.

The aforesaid processes for chrome printing, however, are not fully free from objection on 45 the ground that whilst they are useful in particular instances they do not serve in all cases which come into consideration. Thus they are not suited for printing on mixed fabrics of different fibres.

This invention is based on the observation that 50 good results, such as soft feel, preservation of the lustre of the fibre and even shades can be obtained in printing with mordant dyestuffs on the most varied materials if the printing paste contains 55 lactic acid. This may be used, together with the hitherto usual chromium mordants, such as chromium acetate, and the other usual ingredients, either in the free state or in the form of a salt or ester of lactic acid. Chromium lactate appears to be most suitable; by the use of

this salt a soft feel, a good lustre and even shades are attained under all conditions.

Chromium lactate may be manufactured by general known methods. A preparation suitable for the purpose of the present invention may also be merely obtained from a bichromate and lactic acid whereby the latter serves to reduce the bichromate. 5

The new printing paste gives good results with the different thickenings in printing on vegetable or animal fibres or fibres of regenerated cellulose (artificial silk) or mixed fabrics thereof. Especially remarkable results are obtained in cotton printing, when arabic gum thickening is used. 10

The invention permits the use of a general printing prescription for a large series of mordant dyestuffs which is applicable both for handprinting and printing by machinery and also for the most varied fibres, named above, as well as for 15 all possible mixtures of such fibres.

A further advantage of the present process is a remarkably enhanced stability of the printing pastes accordingly prepared.

The invention provides an improvement of the 25 technique of textile printing which is particularly valuable at the present time, when mixed fabrics play such an important part and when the composition of the fabrics undergoes frequent change at the dictates of fashion.

It will be understood that the process may be 30 combined with any of the known processes, in which urea is used and that the effects obtainable by the known processes, such as those described in U. S. Patent No. 1,848,589, may also be 35 attained in the process of the invention.

It will also be understood that the process is 40 useful not only for direct printing, but also with use of dyestuffs which are resistant to discharge, for colour discharge printing.

The following examples illustrate the invention, the parts being by weight.

## Example 1

There is prepared a printing paste of the following composition:

|                                            | Parts |
|--------------------------------------------|-------|
| Chromocitronine R (Colour Index No. 441) — | 20    |
| Urea —                                     | 50    |
| Water —                                    | 306   |
| Gum arabic thickening 1:1 —                | 600   |
| Chromium lactate containing 14.5 per cent  |       |
| Cr <sub>2</sub> O <sub>3</sub> —           | 24    |
| Total —                                    | 1000  |

Natural silk is printed with this printing paste, dried, steamed for 45 minutes and washed. Prints are obtained in which the silk retains its soft feel and its lustre, whilst the fastness properties do not suffer in any way. Viscose, wool, 60

cotton or any mixed fabrics composed of these fibres can also be printed with the above printing paste with similar results. Instead of chromocitronine R any of the following dyestuffs may be used in preparing the printing paste:

- Chromocitronine 3R (similar to Colour Index No. 442, the dyestuff described in Example 2 of U. S. Patent No. 1,815,827),  
 10 Chromorhodine B (Colour Index No. 762),  
 Chromazurine D (Colour Index No. 879, dyestuff described in Example 1 of U. S. Patent No. 1,895,545),  
 Cuba wood extract (Colour Index No. 1232).  
 15 In all cases the effects above described are attained.

*Example 2*

The following printing paste is prepared:

|                                                                             | Parts    |
|-----------------------------------------------------------------------------|----------|
| 20 Modern violet O (Colour Index No. 892)                                   | 20       |
| Water                                                                       | 336      |
| Acetic acid of 40 per cent strength                                         | 20       |
| Gum thickening 1:1                                                          | 600      |
| 25 Chromium lactate containing 14.5 per cent Cr <sub>2</sub> O <sub>3</sub> | 24       |
| <br>Total                                                                   | <br>1000 |

Viscose or a mixed fabric containing viscose is printed with this printing paste, dried, steamed for 45 minutes, washed and if required soaped. The lustre and feel of the printed fibre are unobjectionable.

*Example 3*

35 The following printing paste is prepared:

|                                                                          | Parts    |
|--------------------------------------------------------------------------|----------|
| Anthacene brown S powder (Colour Index No. 1035)                         | 40       |
| Urea                                                                     | 10       |
| 40 Water                                                                 | 352      |
| Carragheen moss thickening                                               | 550      |
| Chromium lactate containing 14.5 per cent Cr <sub>2</sub> O <sub>3</sub> | 48       |
| <br>Total                                                                | <br>1000 |

Artificial silk or wool is printed with this printing colour, dried and steamed for 45 minutes; the material is then washed and if required subjected to weak soaping. There are obtained brown prints, the fibres having a soft feel.

*Example 4*

55 The following printing paste is prepared:

|                                                                                                                             | Parts    |
|-----------------------------------------------------------------------------------------------------------------------------|----------|
| A mixture of chromocitronine R (Colour Index No. 442 and the dyestuff described in Example 2 of U. S. Patent No. 1,815,827) | 20       |
| 60 Urea                                                                                                                     | 50       |
| Water                                                                                                                       | 230      |
| Gum thickening                                                                                                              | 600      |
| Chromium acetate solution of 20° Bé.                                                                                        | 60       |
| Lactic acid of 50 per cent strength                                                                                         | 40       |
| <br>Total                                                                                                                   | <br>1000 |

A material of viscose, natural silk or of a mixture of these fibres with one another or with other fibres is printed with this printing paste, dried, steamed for 45 minutes and then washed and if required subjected to weak soaping. The yellow-brown prints so obtained have a good feel and lustre and the customary good properties of fastness.

*Examples 5 and 6*

Printing pastes are prepared as follows:

|                                                               | Parts    |
|---------------------------------------------------------------|----------|
| Dyestuff described in Example 2 of U. S. Patent No. 1,888,903 | 30       |
| Chromazurine D (Colour Index No. 879)                         | 30       |
| Water                                                         | 220      |
| Urea                                                          | 130      |
| Furfuryl alcohol                                              | 40       |
| Arabic gum thickening                                         | 550      |
| Chromium lactate with 17% Cr <sub>2</sub> O <sub>3</sub>      | 30       |
| <br>Total                                                     | <br>1000 |

Cotton fabrics are printed with these printing pastes, dried, steamed, for 45 minutes and then washed and eventually soaped.

Thus are obtained prints of a soft feeling which are very sharp even in the finest designs.

What I claim is:

1. In steam printing with chromium mordant dyestuffs on vegetable or animal fibers or fibers of regenerated cellulose, the process for obviating the formation of a harsh feel, uneven dyeing and loss of luster on the imprinted parts caused by coagulation of the thickener in presence of the chromium mordant, comprising printing said material with a paste containing the mordant dyestuffs, gum arabic thickening, and a chromium mordant containing Cr in the cation, in the presence of a lactate group.

2. In steam printing with chromium mordant dyestuffs on vegetable or animal fibers or fibers of regenerated cellulose, the process for obviating the formation of a harsh feel, uneven dyeing and loss of luster on the imprinted parts caused by coagulation of the thickener in presence of the chromium mordant, comprising printing said material with a paste containing the mordant dyestuff, a chromium compound containing Cr in the cation, gum arabic thickening, and lactic acid.

3. In steam printing with chromium mordant dyestuffs on vegetable or animal fibers or fibers of regenerated cellulose, the process for obviating the formation of a harsh feel, uneven dyeing and loss of luster on the imprinted parts caused by coagulation of the thickener in presence of the chromium mordant, comprising printing said material with a paste containing the mordant dyestuff, chromium lactate and gum arabic thickening.

HEINRICH WERDENBERG.

10

5

15

25

30

35

40

45

50

55

60

65